# EUROPEAN PATENT SPECIFICATION

(11) **EP 0 065 421 B1**
(45) Date of publication and mention of the grant of the patent: **28.08.1985**
(21) Application number: 82302504.4
(22) Date of filing: 17.05.1982
(51) Int. Cl.: C25D 11/22, C25D 11/12

(54) **Method of treating a surface of an aluminum to form a pattern thereon**
Verfahren zur Oberflächenbehandlung von Aluminium zur Ausbildung eines Musters darauf
Procédé pour le traitement d'une surface d'aluminium pour former un dessin sur elle

(30) Priority: 19.05.1981 JP 75408/81; 20.05.1981 JP 76313/81
(43) Date of publication of application: 24.11.1982
(73) Proprietor: SANKYO ALUMINIUM INDUSTRY COMPANY LIMITED, Takaoka City Toyama Prefecture 933 (JP)
(72) Inventor: Shima, Isao, Takaoka City Toyama Prefecture (JP); Kazuro Kobayashi, Takaoka City Toyama Prefecture (JP); Ikeda, Yasuzi, Imizu-gun Toyama Prefecture (JP); Sakashita, Mitsuo, Takaoka City Toyama Prefecture (JP)
(74) Representative: Palmer, Roger

## Description

The present invention relates to a method of treating a surface of an aluminum to freely form various patterns thereon.

Throughout the specification, the term "aluminum" used herein means to include aluminum and aluminum alloys.

US-A-4066516 discloses a method of forming a colored pattern on an aluminum or aluminum alloy article, which comprises anodically oxidising the article, forming a barrier layer on those areas not to be colored by a second anodic oxidation step, and electrolytically coloring the article.

As a method of forming a pattern on a surface of an aluminum for buildings having a complicated sectional shape, there have hitherto been proposed various methods wherein the aluminum before an anodic oxidation treatment is dipped into a predetermined electrolytic liquid while applying an electric current thereto (see for instance US-A-4221640).

In these methods, hydrogen gas produced on the surface of the aluminum by the application of electric current rises upward on the aluminum surface to form a bubble-trace pattern. However, the generation of hydrogen gas is not always constant and is very irregular, so that a fixed regular pattern can not be formed on the aluminum surface and also the same pattern can not be reproduced repeatedly.

Moreover, the patterns formed by these methods exclusively relay on the rising trace of hydrogen gas, so that there are obtained only monotonous line and grain-like patterns.

Therefore, the above methods have also a drawback that patterns having appearance and design suitable for various applications can not optionally be obtained.

On the other hand, if it is intended to form a freely designed pattern, usual printing methods are most preferable, but they can not be applied to the aluminum for buildings having a complicated sectional shape.

It is, therefore, an object of the present invention to provide a method of treating a surface of an aluminum to form pattern, which can produce not only a monotonous line pattern but also the same freely designed pattern as in the printing method even on the surface of the aluminum for buildings having a complicated sectional shape.

According to the present invention, there is provided a method of treating a surface of aluminum to form a pattern thereon, which method comprises the steps of electrolyzing the aluminum, after an anodic oxidation treatment, in a bath containing at least one acid or a salt thereof and subjecting the electrolyzed aluminum to electrolytic pigmentation; characterised in that the electrolyzing step is carried out in a bath containing at least one substance selected from the group consisting of organic acids having a hydroxyl or carboxyl group, orthophosphoric acid, pyrophosphoric acid, chromic acid, phosphorous acid, sulphuric amide, highly concentrated sulphuric acid of not less than 40 V/V% and salts thereof in such a manner that the surface of the anodically oxidised aluminum is not sealed during subsequent hot water rinsing of that surface and in that between the electrolyzing step and the electrolytic pigmentation step the electrolyzed aluminum is subjected to a hot water rinsing treatment such that the electrolyzed aluminum is heated thereby to promote the drying of the surface thereof after the rinsing treatment and then a substance for inhibiting or promoting the subsequent electrolytic pigmentation is adhered to the dried surface of the aluminum in a desired pattern, so that in the pigmentation step a pattern based on the difference of color tone between the inhibition or promotion substance adhered portion and the non-adhered portion is formed on the surface of the aluminum.

The aluminum surface after the electrolysis may be subjected to a primary coloration treatment to form a colored anodic oxide film thereon prior to the hot-water rinsing. As the substance contributing to the formation of proper pattern at the subsequent electrolytic pigmentation, there may be used substances capable of inhibiting the electrolytic pigmentation (hereinafter referred to as inhibitation substance) and substances capable of promoting the electrolytic pigmentation (hereinafter referred to as promotion substance).

The present invention will now be described by way of example only in greater detail below.

According to a preferred embodiment of the present invention, the aluminum is first subjected to a pretreatment of degreasing, rinsing, etching and desmutting in a usual manner. The thus treated aluminum is electrolyzed in an electrolytic bath containing sulfuric acid, oxalic acid or a mixture thereof for the production of porous anodic oxide film by a direct current process, an alternating current process, a process of superimposed alternating current to direct current or the other process of using a current wave capable of developing the same effect to form an anodic oxide film on the aluminum surface. Moreover, this anodic oxidation may be accompanied with a color development without interference.

Next, the resulting anodic oxide film of the aluminum is further subjected to an electrolytic treatment, whereby the properties of the anodic oxide film such as structure of micropores and the like are changed.

To this end is used a bath containing at least one of inorganic acids and salts thereof selected from chromic acid, orthophosphoric acid, pyrophosphoric acid, phosphorous acid, sulfuric amide and highly concentrated sulfuric acid of not less than 40 V/V%, or a bath containing at least one of organic acids having a hydroxyl or carboxyl group and salts thereof selected from malic acid, gluconic acid, maleic acid, citric acid, malonic acid, tartaric acid, cresol sulfonic acid, sulfophthalic acid, sulfosalicylic acid, gallic acid, benzoic acid, phthalic acid, carbolic acid and the like. Furthermore, a proper mixture of the above inorganic acid and organic acid may be used as an electrolytic bath.

As a current wave, there are used an alternating current wave, a wave of alternately changing positive and negative polarities, a direct current wave and a superimposed alternating-direct current wave. In the electrolytic treatment, the treating voltage is preferably 5-50 volts and the treating time is 1-10 minutes in order to obtain a sufficient effect. When using the alternating current, the properties of the previously formed anodic oxide film can be largely changed as compared with the case of using the direct current. On the other hand, the use of direct current is small in the range changing the properties the anodic oxide film as compared with the use of alternating current, but has an effect of controlling a current density during the treatment, so that the properties of the resulting colored film become good as compared with the case of using the alternating current.

If necessary, the aluminum may be subjected to a primary coloration treatment after the electrolytic treatment. In this case, any conventional well-known methods can properly be adopted as the primary coloration treatment. For instance, there are mentioned various methods wherein the aluminum is electrolyzed in a coloring bath containing an acid or a salt of a colorable metal selected from nickel, cobalt, copper, tin, manganese, zinc, chromium, iron, molybdenum and the like or further containing hydrogen peroxide by using a proper wave of electric current such as alternating current, direct current, superimposed alternating-direct currents or the like. Alternatively, the aluminum may be colored by a dyeing treatment.

By such a primary coloration treatment, the anodic oxide film is colored into various color tones of bronze, amber, black and the like as well as green, blue, red, yellow, brown and the like.

The subsequent hot-water washing treatment is closely related to the above mentioned electrolytic treatment or primary coloration treatment as apparent from the following reason. That is, it is an essential feature of the present invention that an inhibition substance or promotion substance for subsequent electrolytic pigmentation is adhered to the surface of the anodic oxide film of the colored anodic oxide film according to a desired pattern. Therefore, it is necessary to make the surface of the aluminum into dried state for adhering, the inhibition or promotion substance thereto.

In general, the aluminum is subjected to a rinsing treatment with water after the electrolytic treatment, but it is very difficult to dry the aluminum surface after the rinsing with water. Therefore, a hot-water rinsing treatment is practically preferable in order to increase the production efficiency. However, when the anodic oxide film or the colored anodic oxide film as described above is merely subjected to a hot-water rinsing treatment, the surface of this film is sealed to lose its activity, which prevents the deposition of colorable metal at the subsequent electrolytic pigmentation step.

Therefore, it is necessary to perform the electrolytic treatment for changing the properties of the anodic oxide film as described above in order to ensure the hot-water rinsing treatment without sealing. On the other hand, if the anodic oxide film is subjected to the electrolytic treatment and further to the electrolytic pigmentation without hot-water rinsing, it is certainly colored, but the adhesion of colorable metal is insufficient, so that uniform and beautiful colored anodic oxide film can not be obtained. Therefore, the hot-water rinsing treatment is required for obtaining practically satisfactory films. By the hot-water rinsing treatment, the activity of the anodic oxide film after the electrolytic treatment is made uniform all over the surface of the aluminum, whereby the scattering of metal deposition is prevented at the subsequent electrolytic pigmentation step...

Moreover, when the primary coloration treatment is carried out between the electrolytic treatment and the hot-water rinsing treatment, the properties of the anodic oxide film are never further changed because metal is merely deposited in the micropores or the film is dyed. Therefore, the primary coloration treatment does not adversely affect the subsequent hot-water treatment.

In the hot-water rinsing treatment, pure water is preferably used as a rule, but water containing a surfactant of approximately neutrality or other chemicals may be used. In order to ensure the hot-water rinsing without sealing, the treating time is preferably 1-30 minutes when the treating temperature is 50-90⁰C and 1-15 minutes when the treating temperature is 90―100°C.

When the anodic oxide film or the colored anodic oxide film is subjected to the hot-water rinsing treatment as described above, the surface of the film is made uniform without sealing, so that when the aluminum is taken out from the treating tank, the surface thereof is rapidly made into a dried state. After the hot-water rinsing treatment, the aluminum can be moved to a subsequent treatment of adhering the inhibition or promotion substance for the formation of desired pattern at an electrolytic pigmentation step.

The inhibition substance includes substances flowing no electric current at electrolytic pigmentation step, substances inhibiting the coloring action itself to hardly deposit metal into micropores of the anodic oxide film and the like. As the former substance, mention may be made of kaolin, dibutyl phthalate, acetate, glycerin, ethylene glycol, higher fatty acid esters, insulating substances such as resist ink, synthetic resins and the like. As the latter substance, use may be made of substances producing sodium ion, potassium ion, ammonium ion or nitric acid ion by hydrolysis, an example of which includes aqueous solutions or pastes of sodium hydroxide, potassium hydroxide, ammonia water, nitric acid, sodium nitrate, sodium sulfate, potassium sulfate and the like.

As the promotion substance, use may be made of aqueous solutions of pastes of concentrated sulfuric acid, phosphoric acid, phosphorous acid, sulfuric amide, carboxylic acid, oxycarboxylic acid and the like.

Moreover, the electrolytic pigmentation can be obstructed by using a masking tape.

As a means for adhering the above inhibition or promotion substance to the aluminum surface, there are used direct application of adhesion of these substance as well as various printing processes such as screen printing, off-set printing and the like.

Particularly, it is advantageous to apply the following process to the aluminum having a complicated and irregular surface.

That is, the inhibition or promotion substance is first printed on a thin film according to a predetermined design pattern, which is floated on a liquid upward its printed surface. Then, the aluminum is submerged into the liquid while pushing on the printed surface, whereby the thin film is adhered closely to the overall surface of the aluminum under a liquid pressure to adhere and fasten the inhibition or promotion substance from the printed surface to the aluminum surface. In this case, it is necessary to remove the thin film after the inhibition or promotion substance is adhered to the aluminum surface. Such a removal of the thin film is carried out by various processes such as hot-water rinsing and the like.

After the adhesion of the inhibition or promotion substance at a patterned state, the aluminum surface is subjected to an electrolytic pigmentation treatment. As the electrolytic pigmentation treatment, the conventionally well-known processes can properly be adopted without particular limitation.

For instance, there may be mentioned various electrolytic pigmentation processes wherein the aluminum is electrolyzed in a coloring bath containing an acid or a salt of a colorable metal selected from nickel, cobalt, copper, tin, manganese, zinc, chromium, iron, lead, molybdenum and the like or further containing hydrogen peroxide by using a proper wave of electric current such as alternating current, direct current, superimposed alternating-direct currents or the like. This treatment may be the same as the aforementioned primary coloration treatment. In the latter case, the treating conditions are optionally selected in accordance with desirable colored patterns.

By the electrolytic pigmentation treatment, the anodic oxide film is colored in various color tones such as bronze, amber, black, green, red, blue, yellow, brown and the like irrespective of the previous hot-water rinsing treatment because the properties of the film are previously changed by the electrolytic treatment before the hot-water rinsing.

In the electrolytic pigmentation, when the insulating substance is used as the inhibition substance, the adhered portions are not colored by the electrolytic pigmentation treatment. Therefore, a pattern based on the difference of color tone between the colored portion and the non- colored portion is formed on the aluminum surface.

Moreover, when the primary coloration treatment is previously performed before the electrolytic pigmentation treatment, a colored pattern based on the difference between the color tone in the primary coloration and the color tone in the electrolytic pigmentation is depicted on the aluminum surface.

When the substance inhibiting the coloring action is used as the inhibition substance, the electrolytic pigmentation is not advanced too in the adhered portions, so that there is caused a difference in the coloring degree between the adhered portion and the nonadhered portion. As a result, a colored pattern based on such a difference of the coloring degree is depicted on the aluminum surface.

In case of using the promotion substance, the coloring degree of the adhered portion becomes higher than that of the nonadhered portion, so that the color tone of the adhered portion becomes deeper than that of the nonadhered portion or changes into a different color, whereby a colored pattern is depicted on the aluminum surface.

In the preferred embodiments of the present invention, the activity of the anodic oxide film is uniformized by the hot-water rinsing treatment after the electrolytic treatment, so that the adhesion property of the colorable metal during the electrolytic pigmentation is good and also the coloring degree is uniform all over the irregular surface of the aluminum. Further, there is no limitation for the application of the inhibition or promotion substance to the aluminum surface, so that design patterns can freely be selected and also the same pattern can surely and easily be reproduced.

After the electrolytic pigmentation, the inhibition or promotion substance adhered to the aluminum surface may be left as it is or may be removed in accordance with its nature. In the removal of this substance, the aluminum is subjected to a hot-water rinsing treatment or an immersion treatment in an organic solvent.

The present invention will be described in detail with reference to the following examples.

### Example 1

Aluminum alloy A 6063 S was degreased by immersing in a 10 wt % solution of nitric acid for 5 minutes, etched by immersing in a 5 wt % solution of sodium hydroxide at 50°C for 8 minutes, and desmutted by immersing in a 10 wt % solution of nitric acid. Then, the aluminum alloy was anodically oxidized in a 15 wt % solution of sulfuric acid at a bath temperature of 20°C under a current density of 1.0A/dm2 for 30 minutes and thereafter electrolyzed in a bath containing 100 g/I of phosphorous acid at a bath temperature of 20°C by applying a direct current at 10 volts for 4 minutes. Next, the aluminum alloy was subjected to a hot-water rinsing treatment by immersing in pure water of 80°C for 10 minutes, dried and closely adhered with a water-soluble thin film previously printed by grease according to a desired pattern under a water pressure, whereby grease was adhered to the aluminum alloy surface. The thus treated aluminum alloy was immersed in pure water of 60°C for 15 minutes to remove the water-soluble thin film and then electrolyzed in a bath containing 10 g/1 of stannous sulfate and 10 g/I of sulfuric acid at a bath temperature of 20°C by applying an alternating current at 25 volts for 40 seconds, whereby non-adhered portions were colored green. After the aluminum alloy was immersed in a boiling water for 5 minutes to remove grease, a silver grey-green pattern colored film was formed on the aluminum alloy.

### Example 2

Aluminum plate A 1200 P was subjected to pretreatment and anodic oxidation treatment in the same manner as described in Example 1 and then electrolyzed in a bath containing 55 V/V % sulfuric acid at a bath temperature of 20°C by using it as an anode and applying a direct current at a voltage of 20 volts for 7 minutes. Next, the aluminum plate was subjected to a hot-water rinsing treatment by immersing in pure water of 85°C for 5 minutes, dried, locally covered with a masking tape and electrolyzed in a bath containing 30 g/I of nickel sulfate and 40 gfl of boric acid at a bath temperature of 20°C by using it as a cathode at a voltage of 15 volts for 30 seconds, whereby the noncovered portions were colored lemon gold. After the removal of the masking tape, a beautiful silver grey-lemon gold pattern colored film was formed on the aluminum plate.

### Example 3

Aluminum alloy A 6063 S was subjected to pretreatment and anodic oxidation treatment in the same manner as described in Example 1 and electrolyzed in a bath containing 150 g/I of sulfuric amide and 50 g/I of pyrophosphoric acid at a bath temperature of 25°C by applying a direct current at 15 volts for 5 minutes. Then, the aluminum alloy was subjected to a hot-water rinsing treatment by immersing in pure water of 70°C for 3 minutes, dried, adhered with a mixed solution of dibutyl acetate and vaseline according to a desired pattern and electrolyzed in a bath containing 10 g/I of manganese sulfate and 10 ml/I of hydrogen peroxide at a bath temperature of 20°C. by using it as a cathode at a voltage of 40 volts for 90 seconds, whereby the nonadhered portions were colored brick red. After the adhered substance was removed by immersing in pure water of 100°C for 5 minutes, a silver grey- brick red pattern colored film was formed on the aluminum alloy.

### Example 4

Aluminum plate A 1100 P was subjected to pretreatment and anodic oxidation treatment in the same manner as described in Example 1 and electrolyzed in a bath containing 150 g/l of phosphorous acid and 30 g/I of tartaric acid at a bath temperature of 20°C by using it as an anode and applying a direct current at 15 volts for 2 minutes. Then, the aluminum plate was subjected to a hot-water rinsing treatment by immersing in pure water of 80°C for 4 minutes, dried, adhered with a resist ink by a screen printing process according to a desired pattern and anodically electrolyzed in a bath containing 100 g/I of sulfosalicylic acid and 5 g/I of sulfuric acid at a bath temperature of 20°C at a current density of 2.0 A/dm² for 20 minutes, whereby the nonadhered portions were colored greenish amber. After the resist ink was removed with an organic solvent, a silver grey-greenish amber pattern colored film was formed on the aluminum plate.

### Example 5

Aluminum alloy A 6063 S was subjected to pretreatment and anodic oxidation treatment in the same manner as described in Example 1 and electrolyzed in bath containing 50 g/I of ammonium phosphate and 50 g/I of chromic acid at a bath temperature of 15°C by applying an alternating current at 25 volts for 3 minutes. Then, the aluminum alloy was subjected to a hot-water rinsing treatment by immersing in pure water of 90°C for 3 minutes, dried and coated with a clear lacquer according to a desired pattern. Thereafter, the aluminum alloy was electrolyzed in a bath containing 30 g/I of copper sulfate and 5 g/I of sulfuric acid at a bath temperature of 25°C by applying an alternating current at 20 volts for 2 minutes, whereby the nonadhered portions were colored copper red. After the aluminum alloy was coated with clear lacquer over a whole surface, a beautiful silver grey-copper red pattern colored film was formed on the aluminum alloy.

### Example 6

Aluminum alloy A 6063 S was subjected to pretreatment and anodic oxidation treatment in the same manner as described in Example 1 and electrolyzed in a bath containing 150 g/I of phosphorous acid at a bath temperature of 20°C by applying a direct current at 30 volts for 3 minutes. Then, the aluminum alloy was subjected to a hot-water rinsing treatment by immersing in pure water of 80°C for 4 minutes, dried and printed with a paste of tartaric acid by a screen printing process according to a desired pattern. Thereafter, the aluminum alloy was electrolyzed in a bath containing 10 g/I of stannous sulfate, 30 g/I of nickel sulfate and 20 g/I of cresol sulfonic acid at a bath temperature of 20°C by applying an alternating current at 13 volts for 3 minutes, whereby the paste adhered portions were colored greenish amber and the nonadhered portions were colored gold to form a beautiful pattern colored film on the aluminum alloy.

### Example 7

Aluminum alloy A 6063 S was degreased by immersing in a 10 wt % solution of nitric acid, etched by immersing in a 5 wt % solution of sodium hydroxide at 50°C for 10 minutes, and desmutted by immersing in a 10 wt % solution of nitric acid. Then, the aluminum alloy was anodically oxidized in a 15 wt % solution of sulfuric acid at a bath temperature of 20°C under a current density of 1.0 A/dm² for 30 minutes and electrolyzed in a bath containing 100 g/I of phosphorus acid at a bath temperature of 20°C by applying a direct current at 20 volts for 3 minutes. Thereafter, the aluminum alloy was electrolyzed in a bath containing 30 g/I of nickel sulfate and 30 g/I of boric acid at a bath temperature of 20°C by applying an alternating current at 10 volts for 1 minute, whereby the anodic oxide film was colored greyish blue. Next, the aluminum alloy was subjected to a hot-water rinsing treatment by immersing in pure water of 80°C for 10 minutes, dried and adhered with glycerin according to a desired pattern. Then, the aluminum alloy was electrolyzed in a bath containing 30 g/I of nickel sulfate and 30 g/I of boric acid at a bath temperature of 20°C by applying an alternating current at 15 volts for 5 minutes, whereby the non- adhered portions were colored dark bronze. After glycerin was removed by rinsing with pure water of 90°C for 15 minutes, a greyish blue-dark bronze pattern colored film was formed on the aluminum alloy.

### Example 8

Aluminum alloy A 6063 S was subjected to pretreatment and anodic oxidation treatment in the same manner as described in Example 1 and electrolyzed in a bath containing 200 g/I of orthophosphoric acid and 5 g/I of oxalic acid at a bath temperature of 25°C by applying an alternating current at 15 volts for 5 minutes. Then, the aluminum alloy was electrolyzed in a bath containing 20 g/l of manganese sulfate and 20 ml/I of hydrogen peroxide at a bath temperature of 20°C by using it as a cathode and applying a direct current at 30 volts for 1 minute, whereby the anodic oxide film was colored yellow. Thereafter, the aluminum alloy was subjected to a hot-water rinsing treatment by immersing in pure water of 80°C for 10 minutes, dried and closely adhered with a water-soluble thin film previously printed by dimethyl phthalate according to a desired pattern under a water pressure, whereby dimethyl phthalate was adhered to the aluminum alloy surface. Next, the aluminum alloy was immersed in pure water of 80°C for 20 minutes to remove the water-soluble thin film, dried and electrolyzed in a bath containing 20 g/I of manganese sulfate and 20 ml/I of hydrogen peroxide at a bath temperature of 20°C using it as a cathode and by applying a direct current at 50 volts for 2 minutes, whereby the nonadhered portions were colored dark brown. After the aluminum alloy was immersed in pure water of 80°C for 10 minutes to remove dimethyl phthalate and coated with a clear lacquer, a beautiful yellow-dark brown pattern colored film was formed on the aluminum alloy.

### Example 9

Aluminum plate A 1200 P was subjected to pretreatment and anodic oxidation treatment in the same manner as described in Example 7, electrolyzed in a bath containing 50 V/V % sulfuric acid at a bath temperature of 15°C by applying a direct current at 10 volts for 7 minutes and further electrolyzed in a bath containing 40 g/I of nickel sulfate and 40 g/I of boric acid at a bath temperature of 20°C by using it as a cathode and applying a direct current at 20 volts for 1 minute, whereby, the anodic oxide film was colored gold. Then, the aluminum plate was subjected to a hot-water rinsing treatment by immersing in pure water of 100°C for 5 minutes, dried and coated with a clear lacquer by screen printing process according to a desired pattern.

Next, the aluminum plate was electrolyzed in a bath containing 10 g/I of stannous sulfate and 10 g/I of sulfuric acid at a bath temperature of 20°C by applying an alternating current at 20 volts for 5 minutes, whereby the nonadhered portions were colored black. After the aluminum plate was immersed in pure water of 80°C for 10 minutes and coated with a clear lacquer over a whole surface, a beautiful gold-black pattern colored film was formed on the aluminum plate.

### Example 10

Aluminum alloy A 6063 S was subjected to pretreatment and anodic oxidation treatment in the same manner as described in Example 7, electrolyzed in a bath containing 100 g/i of chromic acid and 5 g/I of sulfuric acid at a bath temperature of 25°C by using it as an anode and applying a direct current at 35 volts, and further electrolyzed in a bath containing 40 g/I of cobalt sulfate and 30 g/I of boric acid at a bath temperature of 20°C by using it as a cathode and applying a direct current at 18 volts for 3 minutes, whereby the anodic oxide film was colored yellowish bronze. Thereafter, the aluminum alloy was subjected to a hot-water rinsing treatment by immersing in pure water of 70°C for 8 minutes, dried and locally adhered with a resist ink. Then, the aluminum alloy was electrolyzed in a bath containing 30 g/I of cobalt sulfate and 20 mill of hydrogen peroxide at a bath temperature by using it as a cathode and applying a direct current at 40 volts for 5 minutes, whereby the nonadhered portions were colored brick red. After the resist ink was removed with an organic solvent, a yellowish bronze-brick red pattern colored film was formed on the aluminum alloy.

### Example 11

Aluminum plate A 1100 P was subjected to pretreatment and anodic oxidation treatment in the same manner as described in Example 7, electrolyzed in a bath containing 80 g/I of sulfuric amide and 50 g/I of pyrophosphoric acid at a bath temperature of 20°C by applying an alternating current at 20 volts for 3 minutes and immersed in an aqueous solution of 10 g/I of ammonium ferric oxalate at 50°C for 1 minute, whereby the anodic oxide film was dyed gold. Thereafter the aluminum plate was subjected to a hot-water rinsing treatment by immersing in pure water at 90°C for 5 minutes, dried and locally adhered with a masking tape. Then, the aluminum plate was electrolyzed in a bath containing 30 g/I of nickel sulfate, 1 g/I of stannous sulfate and 3 g/I of tartaric acid at a bath temperature of 20°C by applying an alternating current at 10 volts for 3 minutes, whereby the nonadhered portions were colored purple. After the removal of the masking tape, a beautiful gold-purple pattern colored film was formed on the aluminum plate.

## Claims

1. A method of treating a surface of aluminum to form a pattern thereon, which method comprises the steps of electrolyzing the aluminum, after an anodic oxidation treatment, in a bath containing at least one acid or a salt thereof and subjecting the electrolyzed aluminum to electrolytic pigmentation; characterised in that the electrolyzing step is carried out in a bath containing at least one substance selected from the group consisting of organic acids having a hydroxyl or carboxyl group, orthophosphoric acid, pyrophosphoric acid, chromic acid, phosphorous acid, sulphuric amide, highly concentrated sulphuric acid of not less than 40 V/V% and salts thereof in such a manner that the surface of the anodically oxidised aluminum is not sealed during subsequent hot water rinsing of that surface and in that between the electrolyzing step and the electrolytic pigmentation step the electrolyzed aluminum is subjected to a hot water rinsing treatment such that the electrolyzed aluminum is heated thereby to promote the drying of the surface thereof after the rinsing treatment, and then a substance for inhibiting or promoting the subsequent electrolytic pigmentation is adhered to the dried surface of the aluminum in a desired pattern, so that in the pigmentation step a pattern based on the difference of color tone between the inhibition or promotion substance adhered portion and the non-adhered portion is formed on the surface of the aluminum.

2. The method according to Claim 1, wherein said aluminum is subjected to a primary coloration treatment between the electrolytic treatment and hot-water rinsing treatment.

3. The method according to Claim 1 or 2, wherein said substance inhibiting the subsequent electrolytic pigmentation is selected from kaolin, dibutyl phthalate, acetate, glycerin, ethylene glycol, higher fatty acid ester, resist ink and synthetic resin.

4. The method according to Claim 1 or 2, wherein said substance inhibiting the subsequent electrolytic pigmentation is selected from aqueous solution and pastes of sodium hydroxide, potassium hydroxide, ammonia water, nitric acid, sodium nitrate, sodium sulfate, ammonium sulfate and potassium sulfate.

5. The method according to Claim 1 or 2, wherein said substance inhibiting the subsequent electrolytic pigmentation is a masking tape.

6. The method according to Claim 1 or 2, wherein said substance promoting the subsequent electrolytic pigmentation is selected from aqueous solution and pastes of concentrated sulfuric acid, phosphoric acid, phosphorous acid, sulfuric amide, carboxylic acid and oxycarboxylic acid.

## Revendications

1. Procédé de traitement d'une surface d'aluminium pour y former un dessin, procédé qui comprend les étapes consistant à électrolyser l'aluminium, après un traitement d'oxydation anodique, dans un bain contenant au moins un acide ou un sel de celui-ci et à soumettre l'aluminium électrolysé à la pigmentation électrolytique, caractérisé par le fait que l'on conduit l'étape d'électrolyse dans un bain contenant au moins une substance choisie dans la groupe comprenant les acides organiques ayant un groupe hydroxyle ou carboxyle, l'acide ortho- phosphorique, l'acide pyrophosphorique, l'acide chromique, l'acide phosphoreux, l'amide sulfurique, l'acide sulfurique très concentré à au moins 40% en volume/volume et leurs sels, de façon telle que la surface de l'aluminium oxydé anodiquement ne soit pas bouchée pendant le rinçage ultérieur de cette surface à l'eau chaude, et par le fait qu'entre l'étape d'électrolyse et l'etape de pigmentation électrolytique, on soumet l'aluminium électrolysé à un traitement de rinçage à l'eau chaude de sorte que l'aluminiuni . électrolysé est chauffé, de manière à favoriser le séchage de sa surface après le traitement de rinçage, et qu'alors on colle à la surface séchée de l'aluminium, en un dessin désiré, une substance servant à inhiber ou à favoriser la pigmentation électrolytique ultérieure, de sorte que dans l'étape de pigmentation, il se forme sur la surface de l'aluminium un dessin basé sur la différence de ton entre la partie où est collée la substance inhibant ou favorisant la pigmentation et la partie où elle n'est pas collée.

2. Procédé selon la revendication 1, dans lequel on soumet l'aluminium à un traitement primaire de coloration entre le traitement électrolytique et le traitement de rinçage à l'eau chaude.

3. Procédé selon l'une des revendications 1 et 2, dans lequel la substance inhibant la pigmentation électrolytique ultérieure est choisie entre le kaolin, le phtalate de dibutyle, l'acétate, le glycérol, l'éthylèneglycol, un ester d'acide gras supérieur, une encre de réserve et une résine synthétique.

4. Procédé selon l'une des revendications 1 et 2, dans lequel la substance inhibant la pigmentation électrolytique ultérieure est choisie entre la solution aqueuse et les pâtes d'hydroxyde de sodium, d'hydroxyde de potassium, l'eau ammoniacale, l'acide nitrique, le nitrate de sodium, le sulfate de sodium, le sulfate d'ammonium et le sulfate de potassium.

5. Procédé selon l'une des revendications 1 et 2, dans lequel la substance inhibant la pigmentation électrolytique est un ruban de masquage.

6. Procédé selon l'une des revendications 1 et 2, dans lequel la substance favorisant la pigmentation électrolytique ultérieure est choisie entre la solution aqueuse et les pâtes d'acide sulfurique concentré, d'acide phosphorique, d'acide phosphoreux, d'amide sulfurique, d'acide carboxylique et d'acide hydroxycarboxylique.

## Patentansprüche

1. Verfahren zur Oberflächenbehandlung von Aluminium für die Ausbildung eines Musters, wobei in aufeinanderfolgenden Schritten das Aluminium nach einer Eloxierbehandlung in einem Bad elektrolysiert wird, das mindestens ein Säure oder ein Salz derselben enthält, und sodann das elektrolysierte Aluminium einer elektrolytischen Pigmentation unterzogen wird, dadurch gekennzeichnet, daß der Elektrolyseschritt in einem Bad durchgeführt wird, das mindestens eine Substanz enthält, die aus der Gruppe von organischen Säuren mit einer Hydroxyl- oder Karboxylgruppe gewählt wird, zu der Orthophosphorsäure, Pyrophosphorsäure, Monochromsäure, monophosphorige Säure, Schwefelsäureamid, hochkonzentrierte Schwefelsäure mit einem Volumenanteil von nicht weniger als 40% sowie deren Salze gehören, dergestalt daß die Oberfläche des eloxierten Aluminiums bei der darauffolgenden Spülung der Oberfläche mit heißem Wasser nicht verdichtet wird, und daß zwischen dem Elektrolyseschritt und dem Schritt der elektrolytischen Pigmentation das elektrolysierte Aluminium einer Spülbehandlung mit heißem Wasser dergestalt unterzogen wird, daß das elektrolysierte Aluminium erhitzt wird, um dadurch die Trocknung der Oberfläche desselben nach der Spülbehandlung zu fördern, und daß sodann eine Substanz zur Förderung oder Hemmung der darauffolgenden elektrolytischen Pigmentation auf die getrocknete Oberfläche des Aluminiums in einem gewünschten Muster aufgebracht wird, so daß beim Pigmentationsschritt auf der Oberfläche des Aluminiums ein Muster entsteht, das durch den Farbtonunterschied zwischen den mit einer fördernden oder hemmenden Substanz beschichteten Bereichen und den unbeschichteten Bereichen bedingt wird.

2. Verfahren nach Anspruch 1, dadurch gekennzeichnet, daß das Aluminium zwischen der Elektrolysebehandlung und der Spülbehandlung mit heißem Wasser einer primären Färbbehandlung unterzogen wird.

3. Verfahren nach Anspruch 1 oder 2, dadurch gekennzeichnet, daß die Substanz, welche die darauffolgende elektrolytische Pigmentation hemmt, aus der Gruppe Kaolin, Dibutylphthalat, Azetat, Glyzerin, Äthylenglykol, höherer Fettsäureester, Reservefarbe und Kunstharz ausgewählt wird.

4. Verfahren nach Anspruch 1 oder 2, dadurch gekennzeichnet, daß die Substanz, welche die darauffolgende elektrolytische Pigmentation hemmt, aus wässerigen Lösungen und Pasten von Natriumhydroxid, Kaliumhydroxid, Ammoniakwasser, Salpetersäure, Natriumnitrat, Natriumsulfat, Ammoniumsulfat und Kaliumsulfat ausgewählt wird.

5. Verfahren nach Anspruch 1 oder 2, dadurch gekennzeichnet, daß die Substanz, welche die darauffolgende elektrolytische Pigmentation hemmt, aus einem Abdeckband besteht.

6. Verfahren nach Anspruch 1 oder 2, dadurch gekennzeichnet, daß die Substanz, welche die darauffolgende elektrolytische Pigmentation fördert, aus wässerigen Lösungen und Pasten von konzentrierter Schwefelsäure, Phosphorsäure, monophosphoriger Säure, Schwefelsäureamid, Karbonsäure und Oxykarbonsäure ausgewählt wird.
